

1

2,743,183

## CHEMICAL SENSITIZATION OF PHOTOGRAPHIC EMULSIONS

Wesley G. Lowe, Jean E. Jones, and Harry E. Roberts, Rochester, N. Y., assignors to Eastman Kodak Company, Rochester, N. Y., a corporation of New Jersey

No Drawing. Application November 8, 1952,  
Serial No. 319,617

1 Claim. (Cl. 95—7)

This invention relates to photographic emulsions and more particularly to chemical sensitizers therefor.

The digestion of washed photographic emulsions, free from silver halide solvents, is known to increase sensitivity without appreciable change in grain size. This process of chemical sensitization was originally ascribed to formation of metallic silver nuclei by reaction of the silver halide with the gelatin or other vehicle. It is now known to be associated in gelatin emulsions primarily with the presence of reactive sulfur compounds which form silver sulfide. It has been demonstrated that sulfites can, under certain conditions such as relatively high silver ion concentration, act as chemical sensitizers and that the product of the reaction of sodium sulfite with silver bromide is probably metallic silver. Also the combined use of reducing agents such as arsenites with sulfur compounds for hypersensitizing has been disclosed. However, there are few specific compounds which have been described as chemical sensitizers other than those reacting to form silver sulfide. Stannous salts and alkali metal stannites, well known for their reducing properties, are described in the literature only as causing fog when used in connection with photographic emulsions for purposes other than sensitizing.

It has been found that under the proper conditions stannous compounds act as chemical sensitizers for photographic emulsions in a manner comparable to sulfur compounds and that this activity can be superimposed on that of sulfur and natural gelatin sensitizers as well as optical sensitizers, particularly the latter, as disclosed in Carroll U. S. Patent 2,487,850.

It has now been found that when silver halide emulsions are sensitized with a sulfur sensitizing agent, a gold salt sensitizing agent and a stannous compound as a sensitizing agent, a speed increase is obtained greater than that expected from the individual effects of the sensitizing agents and greater than that expected from the combined effects of any two of the three types of sensitizing agents.

Therefore, one object of our invention is to provide chemically sensitized emulsions of enhanced light sensitivity. Another object is to provide emulsions having sensitivity enhanced by the combined effect of sulfur, gold and stannous compound sensitizing agents. A further object is to provide the methods of augmenting emulsion sensitivity utilizing the novel combination of sensitizing agents. Further objects of our invention will become apparent from consideration of the following description.

The objects of our invention are accomplished by the incorporation into silver halide emulsions of a mixture of (A) a sulfur sensitizing agent such as disclosed in Sheppard U. S. Patents 1,574,944 granted March 2, 1926, and 1,623,499 granted April 5, 1927, e. g., allyl isothiocyanate, thiocarbamilide, thiourea, sodium thiosulfate, di-o-tolyl thiourea, thioacetamide and allyl thiourea, (B) a gold salt sensitizing agent such as disclosed in Waller and Dodd U. S. Patent 2,399,083, e. g., gold chloride,

2

potassium chloroaurate or an alkali metal aurothiocyanate such as potassium aurothiocyanate and (C) small quantities of stannous compounds such as stannous chloride.

5 The exact type of stannous compound is not especially critical but stannous salts soluble in water but not readily decomposed are preferred, and because of the aerial oxidation of alkali metal stannites, these are less preferred because of the difficulty of obtaining reproducible results. Therefore, acid solutions of stannous salts such as stannous chloride, stannous bromide, iodide, fluoride and sulfate are preferred.

The stannous compounds are used in silver halide emulsions in quantities of the order of from  $1 \times 10^{-7}$  to  $44 \times 10^{-6}$  mol per mol silver halide. When using stannous salts such as stannous halides, we can use a range of concentration of from about  $1 \times 10^{-7}$  to  $20 \times 10^{-6}$  mol per mol silver halide, preferably about  $1 \times 10^{-6}$  to  $9 \times 10^{-6}$  mol per mol silver halide with the faster bromoiodide emulsions of the type shown in the examples below. When using alkali metal stannite solutions made from the stannous salts, we prefer to use from about  $1 \times 10^{-7}$  mol per mol silver halide up to about  $44 \times 10^{-6}$  mol per mol silver halide, the higher quantities sometimes being required when the conditions of operation cause excessive aerial oxidation of the stannite solutions. Generally speaking, the lower ranges of concentration of stannous salts are used with the faster emulsions and up to about  $20 \times 10^{-6}$  mol per mol silver halide with slower fine-grained emulsions except when using stannite solutions. Other factors well known to those skilled in the art will be found to influence the optimum concentration of stannous salt to obtain the characteristics desired for a given photographic emulsion. The appearance of fog with a given emulsion and concentration of stannous salt is a good criterion to follow indicating that too much salt has been used.

The quantities of sulfur and gold salt sensitizing agents in the silver halide emulsions are not especially critical and can be varied from the optimum amounts indicated in the following examples.

The novel sensitizers are incorporated into emulsions at any stage in their preparation but preferably before digestion is complete. That is, the emulsion can first be sensitized with a sulfur sensitizing agent and a gold salt sensitizing agent followed by one of the stannous compounds or the addition of the stannous compound can be made prior to addition of the gold salt. However, it is preferred to partially digest the emulsion in the presence of the selected sulfur and gold salt sensitizing agents and to finish digestion after addition of the stannous compound since the greatest speed increases are obtained in this manner. One rather unexpected feature of our invention resides in the fact that while emulsions can be digested to optimum sensitivity in the presence of sulfur and gold sensitizing agents, further digestion in the presence of the stannous compound does not cause any appreciable increase in fog.

The following example illustrates means of carrying out our invention:

### Example 1

A. In a positive type of silver bromoiodide emulsion were incorporated 20 milligrams of allyl thiourea per mol of silver halide and 2 milligrams of potassium chloroaurate per mol of silver halide and the emulsion was digested for 61 minutes at  $62^\circ\text{C}$ . A sample of the emulsion was coated onto film base.

B. To a sample of emulsion A above were added 0.25 milligram of stannous chloride per mol of silver halide and the emulsion was digested for 20 minutes at  $40^\circ\text{C}$ , before coating on film base.

C. An emulsion was made as in B except using 0.5

milligram of stannous chloride per mol of silver halide. The coatings of emulsions A, B and C were exposed, developed and evaluated sensitometrically with the results shown in the following table:

| Emulsion | Sensitizer                    | 10% Speed | Gamma | Fog  |
|----------|-------------------------------|-----------|-------|------|
| A        | Sulfur+gold                   | 5.50      | 3.30  | 0.04 |
| B        | Sulfur+gold+SnCl <sub>2</sub> | 10.50     | 3.56  | 0.08 |
| C        | Sulfur+gold+SnCl <sub>2</sub> | 11.0      | 3.59  | 0.17 |

A developer of the following composition was used for development of these emulsions:

|                               |       |      |
|-------------------------------|-------|------|
| Water, about 125° F. (50° C.) | cc    | 500  |
| p-Methylaminophenol sulfate   | grams | 2.2  |
| Sodium sulfite, desiccated    | do    | 96.0 |
| Hydroquinone                  | do    | 8.8  |
| Sodium carbonate, desiccated  | do    | 48.0 |
| Potassium bromide             | do    | 5.0  |
| Cold water to make 1.0 liter. |       |      |

*Example 2.*

D. A fine-grained positive type of silver bromoiodide gelatin emulsion was sensitized in a conventional manner with a sulfur sensitizer such as described above, by heating for 30 minutes at 60° C., cooled to 40° C. and coated on film.

E. A sample of the same original emulsion was sensitized in a conventional manner with the sulfur sensitizer used in D and a gold salt sensitizer such as described above, by heating for 30 minutes at 60° C., cooled to 40° C. and coated on film. Upon exposure, processing, and sensitometric evaluation, the emulsion was found to have twice the speed of emulsion D. The combined effect of sulfur and gold salt sensitizing agents is thus illustrated.

F. A sample of the same original emulsion used in D and E was sulfur sensitized in a conventional manner with the same sulfur sensitizer and the same gold salt sensitizer used in E by heating for 30 minutes at 60° C., cooled to 40° C. and 1/2 milligram of stannous chloride per mol of silver halide was added. The emulsion was then held for 20 minutes at 40° C. and coated on film. Upon exposure and processing, this emulsion was found to have twice the speed of emulsion E and four times the speed of emulsion D. This example, as well as Example 1, illustrates enhancing the speed of a sulfur and gold sensitized emulsion by digesting in the presence of a stannous compound.

In processing the emulsions above, development was carried out in a developer of the following composition:

|                               |       |      |
|-------------------------------|-------|------|
| Water about 125° F.           | cc    | 750  |
| p-Methylaminophenol sulfate   | grams | 0.3  |
| Hydroquinone                  | do    | 6.0  |
| Sodium sulfite (desiccated)   | do    | 38.0 |
| Sodium bisulfite              | do    | 1.2  |
| Sodium carbonate (desiccated) | do    | 19.0 |
| Potassium bromide             | do    | 0.9  |
| Citric acid                   | do    | 0.7  |
| Water to 1.0 liter.           |       |      |

In the manner of the above examples, other sulfur sensitizing agents, gold salt sensitizing agents and stannous compounds can be used. When alkali metal stannites are employed to augment sensitivity of sulfur and gold sensitized emulsions, they are simply prepared by dissolving stannous chloride in water and adding sufficient sodium hydroxide to dissolve the oxide first formed. While the above example shows employing digestion after addition of the stannous compound, it is usually not necessary to heat the emulsion after the stannous compound has been added inasmuch as the stannous compounds react very rapidly to enhance emulsion sensitivity.

In the manner of the above examples, many types of silver halide emulsions may be treated with the novel combination of sulfur, gold and stannous sensitizing agents. The novel sensitizers may, in general, be employed in hydrophilic colloid emulsion vehicles; for example, gelatin, polyvinyl alcohol, partially hydrolyzed cellulose esters, such as cellulose acetate and copolymers of polyvinyl alcohol. The sensitizers are suitable for the well known types of silver chloride, silver bromide and silver iodide emulsions and emulsions containing mixtures of these halides, containing the usual emulsion addenda, such as antifoggants, spreading agents, coupler compounds, etc. Such emulsions are suitable to use in forming single as well as multilayer film useful in color photography which customarily include on a support two or more emulsion layers sensitized to different regions of the visible spectrum and may or may not contain coupler compounds. According to our invention such color films carry at least one emulsion layer containing the mentioned combination of sensitizing agents.

Our invention having been described, we would have it understood that the preceding description is by way of example only and that our invention is to be taken as limited only by the scope of the appended claim.

What we claim is:

A light-sensitive photographic emulsion comprising silver halide sensitized with a sulfur sensitizing agent, a gold salt sensitizing agent, and from  $1 \times 10^{-7}$  to  $20 \times 10^{-6}$  mol of stannous chloride per mol of silver halide.

References Cited in the file of this patent

UNITED STATES PATENTS

|           |                   |               |
|-----------|-------------------|---------------|
| 2,399,083 | Waller et al.     | Apr. 23, 1946 |
| 2,487,850 | Carroll           | Nov. 15, 1949 |
| 2,540,086 | Baldsiefen et al. | Feb. 6, 1951  |
| 2,597,856 | Damschroder       | May 27, 1952  |